

## UNITED STATES PATENT OFFICE

1,948,235

ELECTROLYTIC MANUFACTURE OF IRON  
AND ITS ALLOYSErnst Kelsen, Vienna, Austria, assignor to Kelsen  
Special Sheet Holding, S. A., Luxembourg,  
Luxembourg, a limited company of LuxembourgNo Drawing. Application March 17, 1933, Serial  
No. 661,417, and in Austria April 22, 1931

## 2 Claims. (Cl. 204—1)

This invention relates to the electrolytic manufacture of iron and its alloys by means of raw material, e. g. anodes, containing sulphur, and has for its main object to prevent such iron and its alloys from having a sulphur content.

Difficulties are met with in the manufacture of chemically pure iron by electrolytic refining owing to the anode material containing metalloids, such as sulphur and phosphorus, which are present for example when using cast iron scrap. The anodic solution always takes place with a slight overvoltage, so that at least partial oxidation of the sulphur to  $SO_4$ -ion occurs. It is easy to satisfy oneself by analysis that this ion is present in such a refining electrolyte.

The iron raw material, however, is not the only source of sulphur, because both acid and water which must be added throughout the duration of the electro deposition, contains as a rule a 20 certain amount of  $SO_4$ -ion, which also has to be removed.

It is desirable to remove the  $SO_4$ -ion thus formed from the electrolyte, which, when manufacturing iron, consists mainly of ferrous chloride, with or without an additional salt, and which, when manufacturing alloys, consists of salts of those metals of which the alloy consists, also with or without an additional salt, preferably sodium chloride, because, in view of the considerable hydrogen overvoltage at the cathode, the  $SO_4$ -ion undergoes partial reduction, gives up its sulphur content to the electrolytic iron, and thereby impairs the magnetic properties of the latter.

The invention provides a process of reducing the sulphur content of electrolytically manufactured iron or its alloys by an electrolytic refining process employing raw material (e. g. anodes) containing sulphur, characterized in 40 that the electrolyte contains besides the iron salt, or the salts of those metals of which the alloys consist, one or more additional salts whereof at least one gives such a cation, that it gives an insoluble precipitate with  $SO_4$ -ion. Such an 45 additional salt may be added alone as a con-

ducting salt, or it may be added together with another conducting salt.

Conveniently, barium chloride or some other suitable barium salt is added to the electrolyte as a conducting salt. The  $SO_4$ -ion then forms 60 insoluble barium sulphate which readily settles and may be removed from time to time by filtering the electrolyte.

It has heretofore been proposed in certain cases to use  $CaCl_2$  as an additional salt in an 85 iron salt electrolyte. The purpose of adding this salt was, however, quite different from that aimed at by the present invention. The object of adding this salt heretofore was either to improve the electrolytic conductivity or to work 70 at temperatures near or above 100° centigrade, whilst, according to the present invention, the object is to remove from the solution practically the whole content of the  $SO_4$ -ion. For the first mentioned cases it was necessary to add considerable 75 quantities of the salt to attain success, whereas for the purpose of the present invention, a relatively small amount of such a salt is sufficient.

## I claim:

1. In a process of preparing electrolytically manufactured iron of improved magnetic qualities from raw materials containing sulphur, the step of reducing the sulphur content of the electrolytically produced iron by adding to the electrolyte containing the iron salt a salt of an alkaline earth metal which possesses a cation which yields an insoluble precipitate with  $SO_4$ -ion, in an amount sufficient to completely effect such precipitation.

2. In a process of preparing electrolytically manufactured iron of improved magnetic qualities from raw materials containing sulphur, the step of reducing the sulphur content of the electrolytically produced iron by adding barium chloride to the electrolyte containing the iron salt in an amount sufficient to completely precipitate all of the  $SO_4$ -ion.

ERNST KELSEN.